

## UNITED STATES PATENT OFFICE

2,112,468

## PROCESS FOR THE PRODUCTION OF GALVANIZED SHEETS AND THE LIKE

Malcolm E. Morgan, Gadsden, Ala., assignor, by  
means assignments, to Republic Steel Corpora-  
tion, Cleveland, Ohio, a corporation of New  
Jersey

No Drawing. Application March 9, 1936,  
Serial No. 67,914

## 7 Claims. (CL. 148—4)

My invention relates to an improvement in the existing methods employed in the production of galvanized sheets and the like, wherein the rolled sheets are first box annealed and then pickled to 5 prepare them for final treatment in a spelter bath for galvanizing, or in any like bath for the application of a protective surface coating to the sheets.

The finished rolled sheet stock, bearing more 10 or less mill scale, is usually cold rolled to flatten the sheets so they will pile compactly for the box annealing step. As this annealing step proceeds, the mill scale, due to the chemical reaction of its oxygen and the carbon in the sheets, becomes 15 reduced to a residue, in the form of an iron sponge comprising some pure iron and some unreduced oxide of iron, which generally appears in spots on the sheets and, in mill parlance, is referred to as "white oxide". It is resistant to the attack of the pickling solution, and unless removed in the 20 pickling bath, will produce sheets that are graded as "seconds" or "rejects". Therefore, it is the practice, in the effort to maintain the grade of the sheets, to give them a longer pickling treatment to effectively clean them and to apply a 25 heavier spelter coat than would otherwise be necessary. As a result, a reduction in production occurs and there is an increase in acid and spelter consumption per ton of sheets.

I have conceived that if the surface elements 30 of the sheet, which during the annealing step would become reduced to iron oxide or "white oxide", could instead be converted into mainly sulphide of iron, they would then be in a form 35 that is readily removable by the pickle liquor, and as a result I could eliminate the "white oxide", reduce the pickling time required for cleaning sheets, attain material savings of materials in both the pickling and galvanizing steps, and, 40 what is of greatest importance, produce a superior grade of sheets practically free of "seconds" or "rejects".

Broadly expressed, my invention contemplates 45 annealing the sheets in the presence of an agent which will cause the mill scale or other surface portion of the sheet, heretofore reduced to "white oxide", to become converted into mainly sulphide of iron. Such an agent may be a copperas 50 solution with which the sheets are treated before annealing, or sulphuric acid introduced into the annealing box or oven. Both methods produce the same basic reactions on the sheets being annealed in that sulphur gases are liberated which aid in cleaning the sheet surface when the sheets 55 are pickled. Other agents of the order of those

above specified may be employed with similar results.

I prefer to prevent the objectionable reducing action on the surface of the sheets during the box annealing step by wetting the sheet surfaces 5 in any suitable manner, either in whole or in part, with a solution of sulphate of iron or copperas containing two to three pounds of commercial iron sulphate to the gallon of water.

I have put my invention into practice by passing 10 the sheets from the cold rolls through a bath of, or otherwise wetting their surfaces in whole or in part with, 20° Bé. copperas solution, then heat drying the sheets and stacking them preparatory 15 for the box annealing step which proceeds as usual, the annealed sheets being then passed through the pickle bath to clean them before they enter the spelter bath for galvanizing.

I have also successfully practiced my invention 20 by the use of an acid treatment in which about ten pounds of commercial 60° Bé. sulphuric acid is placed in an iron pot under the cover with the sheets during box annealing.

I am also of opinion that like results can be 25 obtained by spraying the copperas solution or pickle liquor on the outer edges of the sheets in the pack ready for the box annealing step.

While the chemical reactions upon which my 30 present method is based are probably complicated, I am of opinion that they proceed in general as follows. In the copperas solution treatment, the copperas dissociates, at box annealing temperatures, into sulphur gases  $SO_2$  and  $SO_3$  which, in the presence of a reducing atmosphere react with the mill scale so that it is readily 35 removable in the acid pickling bath.

In the acid treatment, the acid evaporates and 40 decomposes into  $SO_2$ ,  $SO_3$ , water and oxygen in the annealing box changing the gases therein so that the same reactions occur as when the sheets 45 are dipped. This may be said to produce a preliminary pickling of the sheets prior to annealing, which prepares them for a quicker and more effective cleaning in the final pickle bath that immediately precedes the application of the 45 spelter coat.

I find that by the use of my process I can 50 reduce the pickling time 50%; I can lower the acidity of the pickling bath from 7% at the start to around 5% and effect an acid saving up to 30%; and the sheets come so uniformly gray and clean 55 and free of "white oxide" from the pickling bath that I can effectively galvanize them with a saving of materials running as high as 15 pounds 55

of spelter and 3 pounds of sal ammoniac per ton of sheets.

Having thus described my invention and the preferred methods by which it may be practiced, 5 what I claim as new is:—

1. The herein described step in the method of preparing cold rolled scale bearing finished stock for a galvanizing or like coating step, which consists in wetting the sheet surfaces with a solution 10 of copperas, and then box annealing the treated stock.

2. The herein described steps in the method of preparing cold rolled scale bearing stock for a galvanizing or like coating step, which consists 15 in wetting the sheet surfaces previous to box annealing with a solution of approximately 20° Bé. copperas, and then box annealing the treated stock.

3. The herein described treatment of cold rolled 20 sheet stock, which consists in surface dipping the sheets in a copperas bearing solution, drying them, box annealing the treated stock, pickling the annealed stock, and coating the pickled stock.

4. The herein described step in the preparation 25 of finished ferrous metal sheet stock for galvanizing, which consists in annealing the unpickled stock in an atmosphere containing sulphur dioxide and sulphur tri-oxide.

5. In a process for the production of galvanized ferrous metal sheets, the steps, for the prevention of defects due to the effect of box annealing on mill scale on the sheets, which consist, first, in taking the sheets as they come from the mill and box annealing them in an atmosphere containing a decomposed sulphate in vapor form to react on the mill scale to convert same into a form of iron which is more readily soluble in pickle liquor, and then pickling the annealed 10 sheets.

6. The herein described steps in the method of galvanizing cold-rolled ferrous metal sheets bearing mill scale, which consists in annealing such sheets before they have been pickled in an atmosphere containing sulphuric acid fumes to react with the mill scale during the annealing step, and then pickling the treated sheets.

7. The herein described method for reducing the pickling time required for galvanizing ferrous 20 metal sheets and for reducing the consumption of spelter and pickling acid, which consists in box annealing the unpickled sheets in the presence of vaporized sulphuric acid.

MALCOLM E. MORGAN.